

## UNITED STATES PATENT OFFICE

2,521,926

CHEMICAL SENSITIZATION OF PHOTO-  
GRAPHIC EMULSIONSWesley G. Lowe and Jean E. Jones, Rochester,  
N. Y., assignors to Eastman Kodak Company,  
Rochester, N. Y., a corporation of New JerseyNo Drawing. Application November 18, 1948,  
Serial No. 60,817

11 Claims. (Cl. 95—7)

1

This invention relates to photographic emulsions and more particularly to chemical sensitizers therefor.

It is well known that silver halide emulsions may be chemically sensitized with a variety of materials so as to increase the speed and generally the gamma of the emulsions as opposed to optical sensitizing in which the optical range of sensitivity is increased. Depending upon the materials and methods employed, it is generally regarded that chemical sensitization results in either the formation of silver sulfide on the surface of the silver halide crystal or results in the formation of small amounts of silver from the reduction of silver halide, which effect may be in addition to the former effect usually known as sulfur sensitizing. The present invention is concerned primarily with chemical sensitization apparently of the latter type.

It has been proposed to use organic and inorganic sulfides in photographic emulsions to increase the sensitivity thereof. The compounds are generally regarded as imparting the above-mentioned type of sulfur sensitizing resulting from the formation of silver sulfide nuclei on the silver halide grains. We have discovered a group of organic sulfur-containing compounds which have little or no activity as sulfur sensitizing agents but which appear to depend for their sensitizing effect upon enlargement of the silver sulfide nuclei by deposition of silver thereon through reduction of silver halide. Whatever the mechanism involved, the sensitizing effect is readily distinguishable from ordinary sulfur sensitizing and when employed in conjunction with sulfur sensitizing can be separately evaluated.

One object of our invention is to provide photographic emulsions having increased sensitivities. Another object is to provide emulsions having sensitivities imparted by novel sulfur-containing compounds. A further object is to provide emulsions having sensitivities increased by means of both sulfur sensitizing and the novel sulfur-containing compounds. Another object is to provide sulfur-containing compounds which impart sensitivity to emulsions which effect is distinguishable from the sensitizing effect of ordinary sulfur sensitizers. Other objects of our invention will appear from the following description thereof:

The objects of our invention are accomplished in part by incorporating in silver halide emulsions, either bis-( $\beta$ -aminoethyl) sulfide



and its water-soluble salts obtained from non-desensitizing acids or bis-( $\gamma$ -diethyl aminopropyl) disulfide [ $(\text{C}_2\text{H}_5)_2\text{NC}_3\text{H}_7\text{S—}]\_2$  at any stage in their preparation but preferably before digestion is complete. Generally in order to obtain the optimum sensitizing effect, we heat the emulsion after addition of the sensitizing agent. The sen-

2

sitizing agents may be used in conjunction with other chemical or optical sensitizers such as the well-known sulfur sensitizing compounds disclosed in Sheppard's U. S. Patents 1,574,944, granted March 2, 1926, and 1,623,499, granted April 5, 1927, and may be employed before, after or simultaneously with sulfur sensitizing. Also, our novel sensitizers are useful in conjunction with a variety of emulsions producing pronounced speed increases, particularly with fine-grained positive types of emulsions.

Our invention will now be illustrated by reference to the following specific examples:

## Example 1

15 A 100 cc. sample of a bromo-iodide positive type of emulsion which had previously been peptized with a gelatin derivative and sulfur sensitized with, e. g. allyl thiourea as described in the Lowe et al. U. S. patent application Ser. No. 768,478 filed August 13, 1947, was adjusted to a pH of 6.0. 20 50 mg. of bis-( $\beta$ -aminoethyl) sulfide dihydrochloride were added and the emulsion warmed at 100° F. for two hours, after which 100 cc. of a five 25 per cent solution of gelatin was added. The emulsion was then coated and dried as usual, exposed in an Eastman type 2B sensitometer (J. Soc. Mot. Pict. Eng. 17 (1931) 536) and processed for six minutes in a developer of the following 30 composition:

|                             |        |      |
|-----------------------------|--------|------|
| Water                       | liters | 1    |
| p-Methylaminophenol sulfate | grams  | 0.3  |
| Hydroquinone                | do     | 6.0  |
| Sodium sulfite (dry)        | do     | 38.0 |
| 35 Sodium bisulfite         | do     | 1.2  |
| Sodium carbonate (dry)      | do     | 19.0 |
| Potassium bromide           | do     | 0.9  |
| Citric acid                 | do     | 0.7  |

40 The speed increase is apparent from consideration of the following table (sample D compared to samples A, B and C). Sensitizing the emulsion in the manner described has thus produced a pronounced speed increase appreciably greater than that obtained from the individual sensitizing agents when used alone.

## Example 2

45 A 100 cc. sample of a bromo-iodide positive type of emulsion which had previously been peptized and sulfur sensitized with e. g. allyl thiourea, as disclosed in the Lowe et al. invention, was at this point cooled to 100° F. and adjusted to a pH of 6.0. Two mg. of bis-( $\alpha$ -diethylaminopropyl) disulfide dissolved in acetone solution was then added and the whole allowed to stand at 80° to 90° F. for 1½ hours. The resultant composition was then added to a gelatin solution and coated and dried in the usual manner. After 55 exposure of the emulsion in the sensitometer and development for 6 minutes in the above devel-

oper composition, the emulsion was found to have increased in speed as shown in the table following (sample F compared to E).

In a similar manner, samples of the above emulsion were added to a solution of polyvinyl alcohol and after exposure and processing had the characteristics shown in the table following (sample H compared to sample G). As in the previous example, the sensitizing agent will be seen to have exerted a synergistic sensitizing effect in that the increase in sensitivity is greater than would be expected from the behavior of the individual sensitizing agents when used alone.

| Sample | Sensitizer    | Vehicle           | 10/i Speed | Gamma | Fog  |
|--------|---------------|-------------------|------------|-------|------|
| A      | None          | Gelatin           | 0.58       | 1.18  | 0.01 |
| B      | A*            | do                | 0.78       | 1.54  | 0.02 |
| C      | Sulfur type   | do                | 3.10       | 2.84  | 0.02 |
| D      | Sulfur and A* | do                | 5.20       | 2.94  | 0.02 |
| E      | Sulfur type   | do                | 5.60±      | 3.02  | 0.04 |
| F      | Sulfur and B* | do                | 8.20±      | 3.60  | 0.05 |
| G      | Sulfur type   | Polyvinyl Alcohol | 4.0±       | 2.44  | 0.06 |
| H      | Sulfur and B* | do                | 6.2±       | 3.05  | 0.06 |

\*A=bis-( $\beta$ -aminoethyl) sulfide dihydrochloride.

\*B=bis-( $\gamma$ -diethylamino propyl)disulfide.

±10/E speed at Dens.=0.2 above fog.

In the manner of the above examples, other types of silver halide emulsions may be treated with our novel sensitizing agents alone or in conjunction with other chemical or optical sensitizers. The amount of sensitizing agent used may, depending upon the type of emulsion used, vary somewhat from the optimum amounts employed in the above examples, one-fifth to five times as much sensitizing agent producing emulsions of useful sensitivity. Less heating is usually required when the larger amounts are employed and conversely when using the smaller quantities of sensitizing agent.

It will be noted in the above examples that the sensitizing of the emulsions with the novel sulfide compounds was effected at relatively low pH. This is not a limitation of our invention but more an advantage thereof since we are able to suppress sulfur sensitivity by lowering the pH of the emulsion and since the novel sulfide sensitizers are so active, further sensitization takes place even substantially below the neutral point when they are added to the emulsion.

The novel sensitizers may, in general, be employed in hydrophilic colloid emulsion vehicles; for example, gelatin, polyvinyl alcohol, partially hydrolyzed cellulose esters, such as cellulose acetate and co-polymers of polyvinyl alcohol. The ratio of colloid, to silver halide present during the digestion is not critical in this type of sensitizing since the digestion conditions can be readily adjusted as is well known in the art of sulfur sensitizing. The sensitizers are suitable for the well known types of silver chloride, silver bromide and silver iodide emulsions and emulsions containing mixtures of these halides, containing the usual emulsion addenda such as antifoggants, spreading agents, coupler compounds, etc. Such emulsions are suitable to use in forming single as well as multi-layer film useful in color photography which customarily include on a support two or more emulsion layers sensitized to different regions of the visible spectrum and may or may not contain coupler compounds. According to our invention such color films carry at least one emulsion layer containing a sulfide sensitizing agent of our invention.

Our invention having been described, we would have it understood that the preceding descrip-

tion is by way of example only and that our invention is to be taken as limited only by the scope of the appended claims.

What we claim is:

1. A light-sensitive photographic emulsion comprising silver halide and a sensitizing agent selected from the group consisting of bis-( $\beta$ -aminoethyl) sulfide and water soluble salts thereof, and bis-( $\gamma$ -diethylaminopropyl) disulfide.
2. A light-sensitive photographic emulsion comprising silver halide and bis-( $\beta$ -aminoethyl) sulfide as a sensitizing agent.
3. A light-sensitive photographic emulsion comprising sulfur sensitized silver halide and bis-( $\beta$ -aminoethyl) sulfide as an additional sensitizing agent.
4. A light-sensitive photographic emulsion comprising silver halide and bis-( $\gamma$ -diethylaminopropyl) disulfide as a sensitizing agent.
5. A light-sensitive photographic emulsion comprising sulfur sensitized silver halide and bis-( $\gamma$ -diethylaminopropyl) disulfide as an additional sensitizing agent.
6. The method of increasing the speed of a photographic silver halide emulsion which comprises imparting sulfur sensitivity to said emulsion, adjusting the pH of said emulsion to below neutrality and effecting a further increase in sensitivity by digestion of said emulsion in the presence of a sensitizing agent selected from the group consisting of bis-( $\beta$ -aminoethyl) sulfide and water soluble salts thereof, and bis-( $\gamma$ -diethylaminopropyl) disulfide.
7. The method of increasing the speed of a photographic silver halide emulsion which comprises imparting sulfur sensitivity to said emulsion, adjusting the pH of said emulsion to below neutrality and effecting a further increase in sensitivity by digestion of said emulsion in the presence of bis-( $\beta$ -aminoethyl) sulfide.
8. The method of increasing the speed of a photographic silver halide emulsion which comprises imparting sulfur sensitivity to said emulsion, adjusting the pH of said emulsion to below neutrality and effecting a further increase in sensitivity by digestion of said emulsion in the presence of bis-( $\gamma$ -diethylaminopropyl) disulfide.
9. The method of increasing the speed of a photographic silver halide emulsion which comprises digesting said emulsion in the presence of a sulfur sensitizing agent and a sensitizing agent selected from the group consisting of bis-( $\beta$ -aminoethyl) sulfide and water soluble salts thereof, and bis-( $\gamma$ -diethylaminopropyl) disulfide.
10. The method of increasing the speed of a photographic silver halide emulsion which comprises digesting said emulsion in the presence of a sulfur sensitizing agent and bis-( $\beta$ -aminoethyl) sulfide.
11. The method of increasing the speed of a photographic silver halide emulsion which comprises digesting said emulsion in the presence of a sulfur sensitizing agent and bis-( $\gamma$ -diethylaminopropyl) disulfide.

WESLEY G. LOWE.  
JEAN E. JONES.

#### REFERENCES CITED

The following references are of record in the file of this patent:

| Number  | Country       | Date          |
|---------|---------------|---------------|
| 496,049 | Great Britain | Nov. 21, 1938 |